

3,222,229

**PROCESS OF HARDENING ALLOY STEELS**  
Robert Pribyl, Linz (Danube), Austria, assignor to  
Vereinigte Österreichische Eisen- und Stahlwerke Akti-  
engesellschaft, Linz (Danube), Austria, a firm  
No Drawing. Filed July 30, 1963, Ser. No. 298,535

Claims priority, application Austria, July 14, 1960,

A 5,429/60

10 Claims. (Cl. 148—143)

This application is a continuation-in-part of my co-pending application Serial No. 122,087 filed July 6, 1961, now abandoned, for Process of Hardening Alloy Steels.

This invention relates to hardening alloy steels, which contain about 0.2-0.8% carbon, 0.2-1% silicon, 0.3-2% manganese, 2.1-5% chromium and, if desired, any or several of the following components: 0.2-3% molybdenum, 0.1-0.8% vanadium, up to 9% tungsten, up to 2% cobalt, up to 2% nickel, up to 0.5% titanium and up to 0.5% zirconium.

Most of the steels having these composition ranges are called hot-working steels and are used to make hot-working tools for working metals and the like at elevated temperatures.

Owing to the elevated temperatures of the metals being worked and the temperature changes necessarily involved in each working cycle, hot-working tools are subjected to both mechanical and thermal stresses. These thermal stresses are particularly aggravated in tools, such as hot rolls, which must be cooled during operation. The continually recurring heating and cooling cycles in these tools promote the formation of reticular heat cracks, also referred to as fire cracks. These cracks greatly reduce the life of the tool, and cause the formation of very unclean surfaces on the workpieces.

In order to resist the mechanical and thermal stresses, hot-working steels must have certain performance properties, such as high-temperature stability, high-temperature wear resistance, high-temperature toughness, retention of hardness and freedom from heat cracks. Depending on the nature of the stress, main emphasis must be placed on one property or the other, because it is not possible to combine all the above properties, part of which are mutually inconsistent, in a steel to an equal degree.

These required performance properties can be obtained in steels only if certain alloying elements are used. It is usual to employ chromium, molybdenum, vanadium and tungsten. Molybdenum and tungsten can be substituted either entirely or in part for each other. Nickel is sometimes used to increase toughness. Manganese-silicon steels are often used for lower-grade hot-working tools.

According to the present state of the art, these hot-working steels are hardened, that is, heated and then quenched, only in oil or air. More particularly, as in the case of hot rolls, hardening these steels by water quenching has been impossible owing to the presence and degree of the alloying elements and to the generally large cross-section of such rolls. Thus within these large rolls, water quenching creates sudden, sharp temperature gradients which cause severe internal stresses leading to warping and cracking during treatment.

In accordance with the invention, steels having alloy compositions within the range of 0.2-0.8% carbon, 0.2-1% silicon, 0.3-2% manganese and 2.1-5% chromium, are rapidly heated by any suitable means, to a surface temperature equal to or exceeding the hardening temperature for the specific alloy composition. The steels so heated are subsequently quenched in water, which may be preheated. More particularly, a large steel tool, having an alloy composition within the range

stated, can be thoroughly heated to a moderate, uniform temperature. After the tool has been uniformly heated the surface of the tool is quickly raised to a temperature equal to or greater than the hardening temperature for the specific alloy composition. Water quenching and subsequent tempering complete the process. The tool can be tempered in a furnace, or the like, at suitable temperatures for 60 hours or more to relieve quenching stresses and recover a limited degree of toughness and ductility. The entire process is accomplished without cracking or warping the tool, which would ordinarily occur if the tool was water quenched according to conventional methods of treatment.

Hardening in water results in very high strength tools. For this reason water-hardened steels of the composition described can be more highly tempered, to achieve a certain strength, than tools hardened by the conventional oil or air quenching treatment. The higher tempering is known to improve the resistance to cyclic temperature changes, so that a higher resistance to the formation of heat cracks and consequently an increase of the life of the tool is achieved. The surface quality of the hot-formed workpiece is also increased.

Practical experiments with hot rolls have proved that hardening steels according to the invention improves the quality of the material. The superficial application of heat to the workpiece permits the surface of the steel to be heated above the usual hardening temperatures without detrimental overheating or cracking, which would ordinarily occur if the high temperature deeply penetrated the workpiece. Before hardening, preheating may be arranged, whereby the surface of the workpiece can be raised quickly to a temperature above the usual hardening temperature. The temperature increase beyond the usual value results in a particularly far-reaching solution of the carbides, which are abundantly present in any hot working steel, to improve the retention of hardness. This improvement will be retained even when the increased temperature is allowed to drop to the usual value before quenching.

Detailed information concerning hardening temperatures for specific steel compositions is available in handbooks, industrial standards such as SAE Iron and Steel TR-30, page 190, specifications provided by steel suppliers, and textbooks as, for example, page 301 of the book Tool Steels by Gill, published in 1944 by the American Society for Metals, Cleveland, Ohio.

By experiments it has surprisingly been possible to prove that even heavy hot rolls having, for example, a barrel diameter of 760 mm. and a weight of 6350 kg. and a composition of 0.4-0.5% C, 0.25-0.35% Si, 0.5-0.8% Mn, 2.8-3.3% Cr and 0.1-0.3% V can be quenched with water without danger of cracking when they have been heated to the hardening temperature very rapidly by means of gas-oxygen burners or the like.

A preferred embodiment of the invention may be applied to a workpiece having an alloy composition containing 0.4-0.5% C, 0.25-0.35% Si, 0.5-0.8% Mn and 2.8-3.3% Cr. The steel workpiece is thoroughly and uniformly heated to between 350° C. and 400° C. in a furnace before surface heating. Surface heating is quickly applied by a burner, an electric device, or the like, raising the workpiece surface temperature to between 950° C. and 1010° C. Means may also be used to feed the workpiece at a rate between 37 mm./min. and 50 mm./min. to the burner during the surface heating step. A cooling step, following the surface heating step reduces the workpiece temperature to the range of 860° C. to 910° C. The cooled workpiece is quenched in water having a temperature between 4° C. and 10° C. Stresses caused by quenching are relieved by tempering in a furnace with air circulation for 24 to 36 hours between 400 C. and 630 C.

The final portion of the tempering step can be carried out during a period of 36 hours at between 450° C. and 640° C.

The following are typical examples of the process:

#### EXAMPLE I

##### *Hardening of a hot roll for rolling aluminum*

Size:

|               |     |       |
|---------------|-----|-------|
| Diameter      | mm. | 725   |
| Barrel length | mm. | 1,450 |
| Total length  | mm. | 2,610 |

Composition of the steel:

|    |         |      |
|----|---------|------|
| C  | percent | 0.45 |
| Si | do      | 0.33 |
| Mn | do      | 0.62 |
| Cr | do      | 2.80 |
| Mo | do      | 0.46 |
| V  | do      | 0.16 |

#### STEPS

5

(2) Hardening:

Heating of the workpiece by means of a burner to 980° C.

Quenching temperature 910° C.

Quenching with water having a temperature of 5° C.

(3) Tempering: in a furnace with air circulation for 24 hours at 630° C. and for 36 hours at 640° C.

(4) Hardness after tempering 64-66 Shore-D

#### EXAMPLE IV

##### *Hardening of a mandrel for hot drawing*

Size:

|          |     |       |
|----------|-----|-------|
| Diameter | mm. | 202   |
| Length   | mm. | 1,775 |

Composition of the steel:

|    |         |      |
|----|---------|------|
| C  | percent | 0.50 |
| Si | do      | 0.25 |
| Mn | do      | 0.70 |
| Cr | do      | 3.0  |
| Mo | do      | 0.51 |
| V  | do      | 0.29 |

#### STEPS

25

(1) Heating of the workpiece in a furnace to 350° C.

(2) Hardening:

Heating of the mandrel to 980° C.

Feed speed, 50 mm./min.

Quenching at 910° C. by water having a temperature of 4° C.

(3) Tempering: in a furnace having air circulation for 24 hours at 630° C. and for 36 hours at 640° C.

(4) Hardness after tempering 63-65 Shore-D

#### EXAMPLE II

##### *Hardening of a roll for rolling copper, zinc, tin, brass, lead*

Size:

|               |     |       |
|---------------|-----|-------|
| Diameter      | mm. | 550   |
| Barrel length | mm. | 800   |
| Total length  | mm. | 1,880 |

Composition of the steel:

|    |         |      |
|----|---------|------|
| C  | percent | 0.48 |
| Si | do      | 0.30 |
| Mn | do      | 0.72 |
| Cr | do      | 2.9  |
| Mo | do      | 0.52 |
| V  | do      | 0.22 |

#### STEPS

30

(1) Heating of the roll in a furnace thoroughly to 350° C.

(2) Hardening:

Heating of the roll by means of a burner to 1000° C.

Quenching at 890° C. with water having a temperature of 8° C.

(3) Tempering in a furnace with air circulation for 36 hours at 460° C. and for 36 hours at 520° C.

(4) Hardness after tempering 70-72 Shore-D

#### EXAMPLE III

##### *Hardening of a mandrel for manufacturing of gas bottles by hot drawing*

Size:

|                 |     |     |
|-----------------|-----|-----|
| First diameter  | mm. | 262 |
| Second diameter | mm. | 222 |
| Length          | mm. | 250 |

Composition of the steel:

|    |         |      |
|----|---------|------|
| C  | percent | 0.43 |
| Si | do      | 0.28 |
| Mn | do      | 0.55 |
| Cr | do      | 3.1  |
| Mo | do      | 0.48 |
| V  | do      | 0.20 |

#### STEPS

65

(1) Heating of the mandrel in a furnace thoroughly to 350° C.

(2) Hardening:

Heating of the workpiece by means of a burner to 980° C.

Quenching temperature 910° C.

Quenching with water having a temperature of 5° C.

(3) Tempering: in a furnace with air circulation for 24 hours at 630° C. and for 36 hours at 640° C.

(4) Hardness after tempering 64-66 Shore-D

70

75

the steel alloy composition prior to the step of surface heating said workpiece.

4. A process for hardening alloy steels as defined in claim 3 wherein said workpiece is preheated to a temperature between 350° C. and 400° C.

5. A process for hardening alloy steels as defined in claim 4 wherein said workpiece is tempered at a temperature between 400° C. and 640° C. for a period of from 24 to 60 hours.

6. A process for hardening alloy steels as defined in claim 1 wherein said workpiece is surface heated to a surface temperature between 950° C. and 1010° C.

7. A process for hardening alloy steels as defined in claim 6 wherein said workpiece is cooled to a temperature between 860° C. and 910° C. after the step of surface heating and before the step of quenching said workpiece.

8. A process for hardening alloy steels as defined in claim 7 wherein said workpiece is tempered at a temperature between 400° C. and 640° C. for a period of from 24 to 60 hours.

9. A process for hardening alloy steels as defined in

claim 8 wherein said workpiece is preheated uniformly to a temperature between 350° C. and 400° C. before the step of surface heating said workpiece.

10. A process for hardening alloy steels as defined in claim 9 wherein said workpiece is quenched in water at a temperature between 4° C. and 10° C.

#### References Cited by the Examiner

#### UNITED STATES PATENTS

|           |        |                |       |           |
|-----------|--------|----------------|-------|-----------|
| 1,879,850 | 9/1932 | Klopp          | ----- | 148—152 X |
| 2,070,889 | 2/1937 | Frickey et al. | ----- | 148—143   |
| 2,317,233 | 4/1943 | Taylor         | ----- | 148—152   |
| 2,845,377 | 7/1958 | Seulen et al.  | ----- | 148—150   |
| 2,882,191 | 4/1959 | Van Swaal      | ----- | 148—143   |
| 2,935,433 | 5/1960 | Pribyl         | ----- | 148—144   |

#### OTHER REFERENCES

Tool Steels by Gill, 1944, published by the A.S.M., pages 189, 190, 300, 301, 306 and 482 relied upon.

20

DAVID L. RECK, Primary Examiner.